



US006978533B1

(12) **United States Patent**  
**Yamashita et al.**

(10) **Patent No.:** **US 6,978,533 B1**  
(45) **Date of Patent:** **Dec. 27, 2005**

(54) **METHOD OF MANUFACTURING RARE EARTH-IRON BOND MAGNET**

(75) Inventors: **Fumitoshi Yamashita**, Nara (JP); **Yuichiro Sasaki**, Osaka (JP)

(73) Assignee: **Matsushita Electric Industrial Co., Ltd.**, Osaka (JP)

(\*) Notice: Subject to any disclaimer, the term of this patent is extended or adjusted under 35 U.S.C. 154(b) by 259 days.

(21) Appl. No.: **10/048,644**

(22) PCT Filed: **Aug. 7, 2000**

(86) PCT No.: **PCT/JP00/05273**

§ 371 (c)(1),  
(2), (4) Date: **May 21, 2002**

(87) PCT Pub. No.: **WO01/11636**

PCT Pub. Date: **Feb. 15, 2001**

(30) **Foreign Application Priority Data**

Aug. 6, 1999 (JP) ..... 11-223394

(51) **Int. Cl.<sup>7</sup>** ..... **H02K 15/00**; H02K 15/14; H02K 15/16

(52) **U.S. Cl.** ..... **29/596**; 29/566; 29/602.1; 29/602.2; 29/732; 75/230; 148/101; 148/302; 264/112; 264/122

(58) **Field of Search** ..... 29/596, 602.1, 29/732, 566, 602.2; 141/101, 302; 264/112, 264/122; 75/230; 148/101, 302

(56) **References Cited**

**U.S. PATENT DOCUMENTS**

4,902,361 A \* 2/1990 Lee et al. ..... 148/302  
5,149,477 A \* 9/1992 Yamashita et al. ..... 264/112  
5,300,156 A \* 4/1994 Mohri et al. ..... 148/104

**FOREIGN PATENT DOCUMENTS**

JP 5-94922 4/1993  
JP 6-236807 8/1994  
JP 10-32134 2/1998

**OTHER PUBLICATIONS**

J.F. Herbst et al., "Rare Earth-Iron-Boron Material: A New Era in Permanent Magnets", Ann. Rev. Mater. Sci., 1986, 16, pp. 467-485.

\* cited by examiner

*Primary Examiner*—Carl J. Arbes

*Assistant Examiner*—Tim Phan

(74) *Attorney, Agent, or Firm*—Wenderoth, Lind & Ponack, L.L.P.

(57) **ABSTRACT**

A powder molded magnet manufactured by a method comprising the steps of: (1) forming a granular compound of diameter of not more than 250  $\mu\text{m}$  with a rare earth-iron rapid-quenched flake, which has not more than 150  $\mu\text{m}$  in diameter, being coarsely ground if necessary, and a binder, (2) dry-blending the granular compound with fatty acid metallic soap powder, (3) forming compressed powder from the granular compound dry-blended with the fatty acid metallic soap powder, by powder molding, and (4) heat-treating the compressed powder to a temperature higher than a thermally dissociating temperature of stabilized isocyanate.

**14 Claims, 3 Drawing Sheets**



FIG. 1



FIG. 2



FIG. 3



FIG. 4



FIG. 5



## METHOD OF MANUFACTURING RARE EARTH-IRON BOND MAGNET

### CROSS-REFERENCE TO RELATED APPLICATION

This application is the U.S. National Phase under 35 U.S.C. 371 of International Application PCT/JP00/05273, filed Aug. 7, 2000, which claims priority to Japanese Patent Application No. 11-223394, filed Aug. 6, 1999.

### TECHNICAL FIELD

The present invention relates to a method of manufacturing rare earth-iron bond magnet to form a down-sized thin-arc-shaped magnet with high density and dimensional accuracy. The magnet is used for producing magnetic field in a small DC motor to meet the requirements of higher output power and lower operating current.

### BACKGROUND ART

In the prior art, an arc-shaped magnet used as a field magnet for a small DC motor has been formed mainly of ferrite sintered magnet and ferrite bond magnet, and partly of rare earth-iron bond magnet manufactured by extrusion molding.

Generally, an arc-shaped magnet used as a field magnet is disposed outside of an armature for a small DC motor. A thickness of conventional arc-shaped magnet was not less than 1 mm, no magnet having a thickness of less than 1 mm has been available. When a motor is down-sized, therefore, a motor can not maintain output power since a diameter of an armature must be made smaller. Especially, in case of ferrite magnet, whether it is sintered or bonded, output power of a motor shows remarkable decrease due to the downsizing because enough static magnetic field is not applied to a gap between a field magnet and an armature.

Therefore, a thin-arc-shaped rare earth-iron bond magnet is awaited to provide enough static magnetic field to a gap between an armature and the bond magnet in a small motor.

For down-sizing motors, however, following problems must be solved to manufacture a rare-earth arc-shaped magnet having a wall thickness of less than 1 mm used as a field magnet in a small DC motor.

(1) Poor toughness of a sintered magnet causes breakage or cracks easily. A magnet less than 1 mm thickness is, therefore, hard for being integrated into a motor.

(2) To produce a magnet by injection molding, a molding die cavity must be filled with injected magnetic compound composed of magnet powder and thermoplastic resin. It is difficult, however, to inject magnetic compound having much amount of magnet powder into a molding die cavity of less than 1 mm width.

(3) To produce a magnet by powder molding, a compressed powder is formed first, using magnetic compound composed of magnet powder and thermosetting resin, then heated to cure the compressed powder. It is difficult, however, in powder molding, to fill molding die cavity with the magnetic compound uniformly. Moreover, molding die itself would be damaged due to such a cavity of less than 1 mm width.

(4) To produce a magnet by extrusion molding, extruded magnetic compound composed of magnet powder and thermoplastic resin is cooled just after extruded from a molding die head in case of a magnet of less than 1 mm thickness, which easily causes deformation in the magnet. Therefore, it

is hard to produce a magnet having a wall thickness of less than 1 mm and having dimensional accuracy which allows the magnet to be directly integrated into a motor.

(5) As a method for producing an arc shaped magnet thinner than 1 mm, a machining into less than 1 mm from more than 1 mm thickness may be a solution for a magnet originally formed by injection molding, powder molding or extrusion molding as above mentioned way through 2 to 4. However, machining will easily cause fine cracks, which 10 will make it difficult to integrate the magnet into a motor like the case 1 of a sintered magnet.

Consequently, for the above mentioned thin-arc-shaped magnet, a method of suppressing deformation of magnet is shown in Japanese Patent Non-examined Laid-Open Publication No. H06-236807, disclosing a method of manufacturing comprising the steps of:

- (1) filling a molding die with molten magnetic compound composed of magnet powder and thermoplastic resin; and
- 20 (2) extruding magnetic compound while being cooled the temperature in the molding die below the melting point of thermoplastic resin to prevent deformation.

According to the method disclosed, for example, arc-shaped magnet having a thickness of 0.9 mm can be produced by extrusion molding with a deviation of  $\pm 30 \mu\text{m}$  using magnetic material composed of 95 wt. % of rare earth-iron melt-spun Nd—Fe—B alloy flakes and thermoplastic resin mainly composed of 12-nylon.

In this way, however, magnet characteristics decrease 30 accordingly, compared with a compression-molded magnet, due to reduced volume of magnet powder included because molten thermoplastic resin must act as a carrier of magnetic compound. Furthermore, magnetic material in molding die must be cooled below the melting point of thermoplastics of magnetic compound and solidified in order to form an arc-shaped magnet thinner than 1 mm with dimensional accuracy of not more than  $30 \mu\text{m}$  in thickness deviation. Therefore, the method has drawbacks of molding-die-wear and increase in energy consumption because stronger 40 extruding force is required and extruding speed decreases.

Generally, so-called powder molded magnet includes 45 1.5–3.0 wt. % of resin and has magnet density of 5.9–6.1 g/cm<sup>3</sup>. The magnet is produced using rare earth-iron melt-spun flakes (for example, true-density: 7.55 g/cm<sup>3</sup>) and thermosetting resin (for example, epoxy resin true density: approx. 1.15 g/cm<sup>3</sup>) to form a compressed powder by powder molding, followed by curing by heating thermosetting resin.

On the other hand, magnet density of injection molded or 50 extrusion molded bond magnet is, generally, less than 5.7 g/cm<sup>3</sup>, since much amount of thermoplastics (for example, 12-nylon true density: about 1.1 g/cm<sup>3</sup>), at least 5 wt. %, is needed, which decreases magnet density. A magnetic characteristics of such a magnet is not preferable for a small DC motor to apply a powerful static magnetic field in the gap between an armature and a field magnet, compared with powder-molded magnet, since the characteristics depends only on magnet density.

Therefore, thin-arc-shaped powder molded magnet, with 55 its higher magnet density and dimensional accuracy, has been demanded for a high power permanent magnet motor.

### SUMMARY OF THE INVENTION

This invention has been devised in view of the above-mentioned prior art, aiming to provide a thin-arc-shaped magnet having thickness of less than 1 mm, with high

performance for both dimensional accuracy and magnet density, to provide a gap between a field magnet and an armature of a small DC motor with strong static magnetic field, and its manufacturing method.

In other words, a magnet of this invention is manufactured by a powder molding method basically comprising the steps of

- (1) forming granular compound having a particle-diameter of not more than 250  $\mu\text{m}$ , using binder and rare earth-iron melt-spun flakes having a diameter of not more than 150  $\mu\text{m}$  and coarsely ground if necessary;
- (2) dry-blending the granular compound with fatty acid metallic soap powder;
- (3) forming a compressed powder with the granular compound dry-mixed with fatty acid metallic soap powder, by powder molding; and
- (4) heat-treating the compressed powder to a temperature higher than a thermally dissociating temperature of stabilized isocyanate.

More specifically,

- (1) the magnet powder comprises a rare earth-iron melt-spun flake including  $\text{RE}_2\text{TM}_{14}\text{B}$  (RE denotes Nd and Pr, TM denotes Fe and Co) phase of not more than 300 nm, with specific coercive force  $\text{Hci}$  of 8–10 kOe and residual-magnetization of 7.4–8.6 kG;
- (2) the binder comprises epoxy oligomer which is solid in room temperature and having an alcoholic hydroxyl group in its molecular chain, more specifically, a bisphenol type epoxy oligomer with softening point of 85–95° C.;
- (3) curing agent comprises stabilized isocyanate consisting of one mol of 4-4' diphenylmethane diisocyanate and two-mols of methyl-ethyl-ketone oxime;
- (4) grinding a solid-state block formed by wet blending organic-solvent solutions of those materials and rare earth-iron melt-spun flakes, and then classifying granulate in size.

Furthermore, the fatty-acid metallic-soap powder comprises 100 weight parts of granular compound to which 0.2–0.5 weight parts of calcium-stearate powder is added whose particle diameter is 5  $\mu\text{m}$  or less. Especially, the granular compound is adjusted to have apparent density of 2.7–3.0 g/cm<sup>3</sup> and powder fluidity of 40–45 sec/50 g. A compressed powder having a plurality of arc-shaped sectional views is manufactured, if necessary, for a rare-earth bond magnet having a weight of not more than 0.5 g and the maximum thickness of less than 1 mm. The compressed powder is then heat-treated for not less than 2 minutes at 160–200° C. in the air.

#### BRIEF DESCRIPTION OF THE DRAWINGS

FIG. 1 is a graph showing a relation between a number of 55 grinding times for granular compound having different particle-diameter upper limits and an yield.

FIG. 2 is a graph showing a relation between dimensional accuracy of arc-shaped magnet and a particle-diameter upper limit of granular compound.

FIG. 3 is a graph showing a weight change of compressed powder of continuous powder molding production.

FIG. 4 is a graph showing a demagnetization curve of magnets.

FIG. 5 is a graph showing a relation between a back-side cutting angle and cogging torque.

#### DESCRIPTION OF THE PREFERRED EMBODIMENTS

This invention is aiming at providing a thin-arc-shaped magnet, for example, having thickness of less than 1 mm, with high dimensional accuracy and magnet density, to provide a gap between a field magnet and an armature of a small DC motor with strong static magnetic field and its manufacturing method.

Present invention discloses the fact that an upper limit of particle diameter of granular compound has great influence on dimensional accuracy of a thin-arc-shaped magnet when the granular compound is formed of a uniform mixture of

- (1) magnet powder of rare earth-iron melt-spun flakes,
- (2) a specific epoxy oligomer, and
- (3) a stabilized isocyanate.

Further, present invention discloses production conditions for the granular compound for a stable supply of a thin-arc-shaped magnet having thickness of less than 1 mm in an industrial level.

In other words, the magnet of the present invention is manufactured by a powder molding method basically comprising the steps of:

- (1) forming a granular compound of not more than 250  $\mu\text{m}$  in diameter with rare earth-iron melt-spun flakes having a diameter of not more than 150  $\mu\text{m}$ , the flakes being coarsely ground if necessary, and binder;
- (2) dry-blending the granular compound with fatty acid metallic soap powder;
- (3) forming compressed powder by the granular compound dry-mixed with the fatty acid metallic soap powder, by powder molding; and
- (4) heat-treating the compressed powder to a temperature higher than a thermally dissociating temperature of stabilized isocyanate.

Especially, magnet powder comprises rare earth-iron melt-spun flakes including  $\text{RE}_2\text{TM}_{14}\text{B}$  phase (RE denotes Nd and Pr, TM denotes Fe and Co) of not more than 300 nm, with specific coercive force  $\text{Hci}$  of 8–10 kOe and residual-magnetization of 7.4–8.6 kG. Binder comprises epoxy oligomer, solid at a room temperature, having an alcoholic hydroxyl group in its molecular chain, more specifically a bisphenol type epoxy oligomer with a softening point of 85–95° C. Curing agent comprises stabilized isocyanate consisting of one mol of 4-4' diphenylmethane diisocyanate and two mols of methyl-ethyl-ketone oxime. Pulverizing solid block formed of organic solutions of above materials and rare earth-iron melt-spun flakes in wet process, and following classification provide the granular compound.

Furthermore, fatty-acid metallic-soap powder comprises 100 parts by weight of granular compound to which 0.2–0.5 parts by weight of calcium-stearate powder is added whose particle diameter is not more than 5  $\mu\text{m}$ . Especially, the granular compound is adjusted to have apparent density of 2.7–3.0 g/cm<sup>3</sup> and powder fluidity of 40–45 sec/50 g.

A compressed powder having a plurality of arc-shaped sectional views is manufactured, if necessary, for a rare-earth bond magnet having a weight of not more than 0.5 g and the maximum thickness of less than 1 mm. The compressed powder is then heat-treated for not less than 2 minutes at 160–200° C. in the air.

The rare earth-iron melt-spun flakes used in the present invention are, for example, is in "Rare Earth-Iron-Boron Materials; A New Era in Permanent Magnets" by J. F. Herbst in Ann. Rev. Sci. Vol—16. (1986). The flakes are produced by rapid solidifying a molten alloy containing Nd:Fe:B nearly at a ratio of 2:14:1, and heating properly to

crystallize a  $\text{Nd}_2\text{Fe}_{14}\text{B}$  phase.  $\text{Nd}_2\text{Fe}_{14}\text{B}$  phase is acceptable if it has a single magnetic-domain critical sizes of not more than 300 nm. Magnetically isotropic flakes with residual magnetization  $\text{J}_\text{r}$  of 7.4–8.6 kG and specific coercive force  $\text{H}_\text{ci}$  of 8–10 kOe are preferable.

However, it is also acceptable if the melt-spun flakes include, due to heat treatment, for example, alpha-Fe and nano-composite system including Fe3B type soft magnetism phase and  $\text{Nd}_2\text{Fe}_{14}\text{B}$ , and  $\text{Sm}_2\text{Fe}_{17}\text{N}_3$  type hard magnetism phase or the like.

On the other hand, epoxy oligomer having an alcoholic hydroxyl group in molecular chain and is solid at a room temperature such as bisphenol type epoxy oligomer and stabilized isocyanate are used to bind above-mentioned magnet fine particles with much stronger adhesion. As the stabilized isocyanate is an isocyanate compound added with active-hydrogen compound beforehand, the isocyanate group released by thermal dissociation reacts with an alcoholic hydroxyl group to cross-link by a urethane bond.

In this case, a part of released isocyanate group reacts with water adsorbed on magnet fine-particle (metal) surface, and form a substituted urea compound and make a chelate bonding with metallic-oxide surface. Furthermore, since thermal dissociation of stabilized isocyanate does not occur at a room temperature below 40°C., polymerization reaction with epoxy oligomer does not occur even if the stabilized isocyanate is uniformly mixed with epoxy oligomer. In other words, magnet powder containing granular compound can be adjusted to maintain the inactive condition which does not change powder-moldability after storage for several years.

The present invention is explained by following embodiments more in detail. However, this invention is not limited to the embodiments.

#### [Magnet Powder and its Coarse Grinding]

Magnet powder used in this invention is a product from Magnequench International In, Co. (Trade Mark: MQP-B), which is a rare earth-iron melt-spun flake with a thickness of 20–30  $\mu\text{m}$  and having alloy composition of  $\text{Nd}_{12}\text{Fe}_{77}\text{Co}_5\text{B}_6$ , and magnetically isotropic  $\text{Nd}_2\text{Fe}_{14}\text{B}$  phase with crystal particles having a diameter of 20–50 nm. The magnet powder contains 39.7% particles in weight which passes 150  $\mu\text{m}$  sieve at their initial conditions. Subsequently, 10 kg of magnet powder, not smaller than 150  $\mu\text{m}$ , is ground at 1312 r.p.m. in a 20 liter Henschel mixer for 5 minutes in a nitrogen atmosphere.

Table 1 shows yield of magnet powder not greater than 150  $\mu\text{m}$  and number of coarse-grinding time for magnet

pressed powder formed by powder molding, pulverized powder not greater than 53  $\mu\text{m}$  is seldom produced, as clearly shown in Table 1.

TABLE 1

| 10 | Particle Diameter<br>( $\mu\text{m}$ ) | Number of Coarse Grinding Time |       |       |       |
|----|----------------------------------------|--------------------------------|-------|-------|-------|
|    |                                        | Initial                        | 1     | 2     | 3     |
| 15 | <53                                    | 3.44                           | 1.58  | 1.00  | 1.91  |
|    | 53–75                                  | 9.49                           | 3.77  | 2.39  | 4.37  |
|    | 75–106                                 | 18.92                          | 8.98  | 5.77  | 9.10  |
|    | 106–125                                | 28.07                          | 20.65 | 15.92 | 20.10 |
|    | 125–150                                | 39.69                          | 51.62 | 37.91 | 40.50 |
|    | 150–250                                | 85.73                          | 99.00 | 99.60 | 99.58 |
|    | 250–350                                | 99.79                          | 99.98 | 100.0 |       |
|    | Yield<br>(<150 $\mu\text{m}$ )         | 39.7%                          | 70.8% | 81.9% | 89.2% |
|    |                                        |                                |       |       |       |
|    |                                        |                                |       |       |       |

#### [Preparations of Binder Composition]

7 kinds of bisphenol type epoxy oligomers as shown in Table 2 and chemical formula 1, each having different melting point, and stabilized isocyanate which consists of one mol of 4-4' diphenylmethane diisocyanate and two-mols of methyl-ethyl-ketone oxime as shown in chemical formula 2 are dissolved in acetone to make an acetone solution of 50% concentration. The ratio between –NCO group of an stabilized isocyanate and sum of the alcoholic hydroxyl group in molecular chain of bisphenol type epoxy oligomer is specified as 0.8.

TABLE 2

| 40 | Sample | Degree of polymerization | Molecular Weight | Epoxy equivalent | Melting point |
|----|--------|--------------------------|------------------|------------------|---------------|
| 45 | A      | 0.1                      | 380              | 190              | Liquid        |
|    | B      | 2.0                      | 900              | 500              | 65–75         |
|    | C      | 2.6                      | 1060             | 650              | 75–85         |
|    | D      | 3.7                      | 1400             | 950              | 95–105        |
|    | E      | 8.8                      | 2900             | 2250             | 115–125       |



powder not smaller than 150  $\mu\text{m}$ . As clear from the table, the yield reaches to not less than 90% by repeating coarse-grinding three times or more. Moreover, although too finely ground magnet powder causes a density decrease in com-

#### [Preparation of Granular Compound]

95 weight % magnet powder, not greater than 150  $\mu\text{m}$  and 2.5 weight % acetone solution of epoxy resin are mixed in wet process using a sigma blade type kneader. Subse-

quently, the mixture is heated at 80–90° C. to evaporate acetone to obtain a solid block at a room temperature. The block is ground into granule by a cutter mill, and the granule is classified directly by sieves of 500, 350, 250, 212 and 150  $\mu\text{m}$  respectively.

FIG. 1 shows a relation between a number of grinding times for granular compound and an yield, varying particle-diameter upper limit of 500, 350 and 250  $\mu\text{m}$  respectively. Where, line A in the figure shows a relation between the number of grinding times and the yield for the granular compound having particle-diameter upper limit of 250  $\mu\text{m}$ . The granular compound is formed by grinding a solid block comprising magnet powder, not greater than 150  $\mu\text{m}$  as disclosed in the present invention, and epoxy resin using bisphenol type epoxy oligomer (melting point: 95–105° C.). On the other hand, lines B–D show a number of grinding times and yields for granular compound having particle-diameter upper limit of 500, 350 and 250  $\mu\text{m}$ . The granular compounds are formed by grinding a solid block comprising magnet powder, in which 60.3 weight % of particles are not smaller than 150  $\mu\text{m}$  (See Table 1) and epoxy resin using bisphenol type epoxy oligomer (melting point: 95–105° C.).

As is clearly shown in the figure, granular compound having particle-diameter upper limit of 250  $\mu\text{m}$ , as disclosed in the present invention, can be obtained in good yield by using the magnet powder upper limit of 150  $\mu\text{m}$ . Additionally, in the example explained below, magnet powder, not greater than 150  $\mu\text{m}$  is used to form granular compound having the particle diameter upper limit of 250, 212 and 150  $\mu\text{m}$  respectively.

#### [Effect of Fatty-Acid Metallic Soap]

The granular compounds, having the particle-diameter upper limit of 500, 350 and 250  $\mu\text{m}$  each, are uniformly mixed with 0.2–0.6 parts by weight of fatty-acid metallic soap at a temperature below 40° C. with a V shaped mixer.

The effects of fatty-acid metallic soaps are evaluated on 100 parts by weight of granular compound having 250  $\mu\text{m}$  of particle-diameter upper limit using bisphenol type epoxy oligomer (melting point: 95–105° C.) by adding 0.2–0.6 parts by weight of stearic acid, zinc stearate, calcium stearate, aluminum stearate, and magnesium stearate respectively. Consequently, calcium-stearate powder, not greater than 75  $\mu\text{m}$ , shows preferable increase in fluidity of granular compound most, little change in apparent density after storage, and comparatively few reduction in radial crushing strength. On the other hand, calcium-stearate powder, not smaller than 75  $\mu\text{m}$  is not suitable because it easily separates from granular compound. Stearic acid and zinc stearate are not suitable since both have lower melting points than the curing temperature (160° C.) and show, especially, large decrease in radial crushing strength.

#### [Melting Point and Moldability of Bisphenol Type Epoxy Oligomer]

Table 3 shows a relation between a melting point of bisphenol type epoxy oligomer and apparent density (JIS Z2504) and fluidity (JIS Z2502) of a granular compound having particle-diameter upper limit of 250  $\mu\text{m}$ , which include 0.2 parts by weight of calcium-stearate powder as fatty-acid metallic soap. As shown in the table, the compound using the bisphenol type epoxy oligomer, liquid at room temperature, has poor fluidity. However, every granular compound using bisphenol type epoxy oligomer, which is solid at a room temperature, shows an acceptable powder fluidity for powder molding. Then, 1 kg of these compounds is calmly filled into steel containers with a bore of 50 mm

respectively, and the apparent density and fluidity of each compound after 240 hours at 40° C. are investigated.

As a results, although bisphenol type epoxy oligomer, having the melting point of below 75–85° C., shows little change in fluidity, apparent density changes to 2.95–3.05 g/cm<sup>3</sup> from initial value of 2.75. In other words, bisphenol type epoxy oligomer having a melting point of higher than 95–105° C. is preferable for granular compound used in 10 powder molding with high dimensional accuracy.

On the other hand, as to magnet density and radial crushing strength also shown in Table 3, bisphenol type epoxy oligomer with the melting point below 95–105° C. shows preferable results. Where, density (JIS Z2505) and radial crushing strength (JIS Z2507) are measured for bond magnet which is manufactured the following steps:

- (1) filling an ring shape mold cavity having an outer diameter of 12.8 mm and an inner diameter of 10.5 mm with granular compound;
- (2) applying pressure of 8 ton/cm<sup>2</sup> to form a compressed powder of 10 mm height; and
- (3) heating the compressed powder for 2 minutes at 160° C.

TABLE 3

| Melting temperature of oligomer (° C.)         | Liquid | 65–75 | 75–85 | 95–105 | 115–125 |
|------------------------------------------------|--------|-------|-------|--------|---------|
| Fluidity (sec/50 g)                            | 57.2   | 44.1  | 41.3  | 40.9   | 40.5    |
| Apparent density (g/cm <sup>3</sup> )          | 2.23   | 2.75  | 2.75  | 2.85   | 2.85    |
| Magnet density (g/cm <sup>3</sup> )            | 6.1    | 6.0   | 6.0   | 6.0    | 5.9     |
| Radial crushing strength (kg/mm <sup>2</sup> ) | 5.04   | 4.87  | 4.67  | 4.76   | 3.67    |

#### [Curing Conditions for Bond Magnet]

Table 4 shows radial crushing strength at a room temperature on bond magnet manufactured by the following steps:

- (1) Adding 0.2 parts by weight of calcium-stearate to 100 w/t parts of granular compound, having a particle-diameter upper limit of 250  $\mu\text{m}$ , using bisphenol type epoxy oligomer (melting temperature: 95–105° C.);
- (2) filling an ring shape molding die cavity having outer diameter of 12.8 mm and a inner diameter of 10.5 mm with the granular compound to form compressed powder of 10 mm height by applying compression of 8 ton/cm<sup>2</sup>; and
- (3) heating the compressed powder for 2–20 minutes at 80–200° C.

Radial crushing strength becomes four times larger than compressed powder by heating for 2 min at, for example, 160° C. using a system comprising a bisphenol type epoxy oligomer and stabilized isocyanate which consists of one mol of 4-4' diphenylmethane diisocyanate and two-mols of methyl-ethyl-ketone oxime. In addition, the same level of radial crushing strength requires 20 minutes heating at 130° C. Therefore, preferable curing conditions for bond magnet of the present invention is to heat for more than 2 minutes at 160–200° C.

TABLE 4

| Time<br>(min.) | Curing Temperature (° C.) |                |                |                |                |                |                |                |
|----------------|---------------------------|----------------|----------------|----------------|----------------|----------------|----------------|----------------|
|                | 80                        | 100            | 120            | 130            | 140            | 150            | 160            | 200            |
| 2              | 1.17<br>(1.01)            | 1.74<br>(1.51) | 2.68<br>(2.33) | 2.82<br>(2.44) | 2.40<br>(2.09) | 4.42<br>(3.84) | 4.81<br>(4.18) | 4.85<br>(4.21) |
| 5              | 1.22<br>(1.06)            | 1.90<br>(1.65) | 2.51<br>(2.18) | 2.93<br>(2.54) | 4.34<br>(3.77) | 5.19<br>(4.51) | 5.05<br>(4.39) | 4.88<br>(4.24) |
| 10             | 1.33<br>(1.15)            | 2.29<br>(1.99) | 3.04<br>(2.64) | 3.27<br>(2.84) | 4.99<br>(4.34) | 5.65<br>(4.91) | 5.59<br>(4.86) | 5.17<br>(4.50) |
| 20             | 1.51<br>(1.31)            | 2.36<br>(2.05) | 3.88<br>(3.37) | 4.81<br>(4.18) | 5.41<br>(4.70) | 5.70<br>(4.95) | 5.62<br>(4.89) | 5.15<br>(4.48) |

Unit in kg/mm<sup>2</sup>. Values in brackets show ratios to compressed powder as 1

15

[Relation between Particle-Diameter Upper Limit of Granular Compound and Dimensional Accuracy of Thin-Arc-Shaped Compressed Powder]

FIG. 2 is a graph, in which deviation in thickness of arc-shaped compressed powder are plotted for each particle-diameter upper limit after heated to cure for 2 min. at 160° C. Compressed powder is formed of 100 parts by weight of granular compound, having particle-diameter upper limit of 500, 350, 250, 212 and 150 μm respectively, using bisphenol type epoxy oligomer (melting point: 95–105° C.) to which 0.2 parts by weight of calcium-stearate is added.

Where, magnet dimensions are outer radius of 3.65 mm, inner radius of 3.55 mm, the maximum thickness of 0.90 mm and length of 15.5 mm.

After molding die cavity is filled with granular compound, molding die is raised up over the thickness (1.75 mm) of whole arc-shaped magnet to make granular compound sink into molding die cavity, which is so-called under-filling operation in powder molding. Then the granular compound is compressed by 8 ton/cm<sup>2</sup> to form a compressed powder. Furthermore, the compressed powder is released from molding die while keeping held by upper and bottom punches. A curvature dimension of molding die is exactly transferred on the compressed powder, since these dimensions are exactly transferred by preventing rebound action of spring-back, when compressed powder is released in above described powder-molding condition.

Now, deviation range of ±3 A μm of an arc-shaped magnet thickness and particle-diameter upper limit P of a granular compound are in the relation of following equation (the correlation coefficient of regression is 0.988).

$$A = 0.0003P^2 - 0.0718P + 24.745$$

As is clear from the figure and regression equation, if a particle-diameter upper limit of a granular compound is not more than 250 μm, thickness deviation of the thin-arc-shaped magnet with a wall thickness of less than 1 mm will become not more than ±30 μm or even not more than ±26 μm. The technical problem pointed out by JPO6-236807, i.e., the difficulty of uniform filling of the magnet powder (or the granular compound in the present invention) into molding cavity, is solved by the present invention.

On the other hand, as an example for comparison, a thin-arc-shaped magnet having the same dimensions is manufactured by the same method indicated by JPO6-236807, as follows:

(1) kneading magnetic compound composed of 5 weight % of 12-nylon and 95 weight % of magnet powder whose particle diameter is less than 150 μm as the same particle diameter as disclosed in this invention, at 260° C.,

(2) forming a pellet using the magnetic compound,  
(3) manufacturing a thin-arc-shaped magnet using the pellet, setting the molding die head temperature at 175° C., which is below the melting point of 12-Nylon, by extrusion molding method.

The deviation in thickness at the maximum thickness portion of 0.9 mm is ±30 μm. Consequently, according to the present invention, a thin-arc-shaped magnet with equal or higher dimensional accuracy than extrusion molding can be manufactured by powder molding, which is once denied due to a difficulty in the above Publication.

[Weighing Accuracy for Continuous Powder Molding]

FIG. 3 is a graph, in which weights of arc-shaped compressed powder are plotted for 250 times continuous powder molding production at each molding shot. The compressed powder is formed of 100 parts by weight of granular compound, having particle-diameter upper limits of 250 μm, using bisphenol type epoxy oligomer (melting point: 95–105° C.) to which 0.2 parts by weight of calcium-stearate is added.

Where the magnet dimensions are outer radius of 3.65 mm, inner radius of 3.55 mm, the maximum thickness of 0.90 mm and length of 15.5 mm. After a molding-die-cavity is filled with granular compound, the molding die is raised up over the thickness (1.75 mm) of whole arc-shaped magnet to make granular compound sink into the molding-die-cavity, which is so-called under-filling operation in powder molding. Then the granular compound is compressed by 8 tons/cm<sup>2</sup> to form compressed powder. Furthermore, the compressed powder is released from the molding die while keeping held by upper and bottom punches.

In the figure, straight lines A and A' show 0.4636 g and 0.4379 g respectively, which correspond to weight threshold values of ±30 μm deviation for the maximum thickness of 0.9 mm of arc-shaped magnet. Actual weighing shows the maximum value of 0.461 g, the minimum value of 0.448 g, resulting in only 13 mg of difference. In other words, it is obvious that thin-arc-shaped magnet of under 1 mm thickness can be manufactured in a stable condition in industrial volume by powder molding method of the present invention.

[Magnetic Characteristics of Magnet]

A rare earth-iron bond magnet having a cylindrical shape of 5 mm in diameter and 5 mm length is provided by powder molding a compressed powder, pressed by 8 tons/cm<sup>2</sup> followed by a heat-treatment for 2 minutes at 160° C. The compressed powder is formed of 100 parts by weight of granular compound, having particle-diameter upper limits of 250 μm, using bisphenol type epoxy oligomer (melting point: 95–105° C.) to which 0.2 parts by weight of calcium-stearate is added. Then, applying pulse magnetization of 50

## 11

kOe in height direction of the cylinder-shaped magnet, a demagnetization curve is obtained using vibration sample-type magnetometer (VSM) at a measurement magnetic-field of  $\pm 20$  kOe. Further, the extrusion molded magnet is formed by melting and curing the pellet which include 95 weight % of magnet powder and 5 weight % of 12-nylon and is kneaded at 260° C., and the demagnetization curve is also obtained. FIG. 4 is a graph showing the demagnetization curve of so-called compression molded magnet formed of powder molding and heat-treatment of compressed powder of the present invention, and that of the extrusion molded magnet for a comparison. Table 5 shows the magnetic characteristics obtained from the demagnetization curves.

As is obvious from FIG. 4 and Table 5, the embodiment of the present invention shows higher magnetic characteristics compared with the comparative example. Supposedly, this is because high filling ratio of magnet powder is possible in powder molding method of the invention. On the other hand, too finely pulverized and oxidized magnetic material kneaded with a strong shearing force at a high temperature of 260° C. may decrease the magnetic characteristics of the comparative example.

TABLE 5

|                     | Specific Coercive force Hci kOe | Residual magnetization $4 \pi M_r$ kG | Maximum energy product $[BH]_{max}$ MGOe | Squareness Hk |
|---------------------|---------------------------------|---------------------------------------|------------------------------------------|---------------|
| Present invention   | 9.53                            | 6.87                                  | 9.55                                     | 2.59          |
| Comparative Example | 8.66                            | 6.58                                  | 8.30                                     | 2.24          |

[Advantages of Arc-Shaped Magnet with a Plurality of Sectional Shapes Longitudinally]

An extrusion molding method as disclosed in JP 06-236807 can not provide an arc shaped magnet with a plurality of sectional shapes longitudinally. However, a thin-arc-shaped magnet used as a field magnet for a small DC motor, the subject of this invention aiming, is required to apply strong static magnetic field in a gap between the field magnet and an armature to satisfy both down-sizing and higher power output of a motor. On the other hand, cogging torque must be low enough for an armature to rotate smoothly. Although an armature having portions of different diameters may be one solution to lower the cogging torque, it will result in increasing an operating current easily by magnetic saturation in an iron core.

A powder molding, therefore, of the present invention, can provide an arc-shaped magnet with more than two kinds of sectional shapes longitudinally by designing an upper and a lower punches arbitrarily. With such a magnet, magnetic resistance in magnetic pole surface can be varied with respect to a rotating direction of an armature, and cogging torque can be reduced by shaping a molded magnet appropriately. FIG. 5 shows a relation between a back-side cutting-angle and cogging torque of an arc-shaped magnet where a part of outer surface of the magnet has a cut portion.

## INDUSTRIAL APPLICABILITY

The present invention provides a method of manufacturing a thin-arc-shaped magnet having a thickness of less than 1 mm, with high dimensional accuracy and magnet density. The magnet provides, for example, a gap between a field magnet and an armature of a small DC motor with strong

## 12

static magnetic field. Of course, it is needless to say that the present invention can be applied for various shapes of magnet other than a thin-arc-shaped magnet with a thickness of less than 1 mm.

5 What is claimed is:

1. A method for manufacturing an arc-shaped rare earth-iron bond magnet having a weight of not more than 0.5 g and a thickness of less than 1 mm, the method comprising the steps of:

- 10 (1) grinding rare earth-iron melt-spun flakes to a diameter not greater than 150  $\mu$ m;
- (2) forming a granular compound by blending the rare earth-iron melt-spun flakes not greater than 150  $\mu$ m in diameter with an epoxy oligomer and a stabilized isocyanate curing agent;
- (3) grinding and classifying the granular compound to have a particle diameter of less than 250  $\mu$ m;
- (4) dry blending the granular compound having a particle diameter of less than 250  $\mu$ m with fatty acid metallic soap powder;
- (5) compressing a powder comprising the blend of the granular compound and the fatty acid metallic soap powder in an arc-shaped mold to form a compressed powder; and
- (6) heat-treating the compressed powder to form the arc-shaped rare earth-iron bond magnet having a weight of not more than 0.5 g and a thickness of less than 1 mm.

20 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 973

**13**

13. A rare earth-iron bond magnet produced by the method according to claim 1.

14. A small DC motor comprising an arc-shaped magnet produced by the method of claim 1, said magnet having a weight of not more than 0.5 g and a thickness of less than 1 mm, wherein said magnet is produced by the steps of:

- (1) grinding rare earth-iron melt-spun flakes to a diameter not greater than 150  $\mu\text{m}$ ;
- (2) forming a granular compound by blending the rare earth-iron melt-spun flakes not greater than 150  $\mu\text{m}$  in 10 diameter with an epoxy oligomer and a stabilized isocyanate curing agent;
- (3) grinding and classifying the granular compound to have a particle diameter of less than 250  $\mu\text{m}$ ;

**14**

(4) dry blending the granular compound having a particle diameter of less than 250  $\mu\text{m}$  with fatty acid metallic soap powder;

(5) compressing a powder comprising the blend of the granular compound and the fatty acid metallic soap powder in an arc-shaped mold to form a compressed powder; and

(6) heat-treating the compressed powder to form the arc-shaped rare earth-iron bond magnet having a weight of not more than 0.5 g and a thickness of less than 1 mm.

\* \* \* \* \*